

Oct. 8, 1929.

C. ELLIS

1,731,194

COVER FOR BOTTLE STOPPERS

Filed May 9, 1925



*Inventor*  
*Charles Ellis*

## UNITED STATES PATENT OFFICE

CARLETON ELLIS, OF MONTCLAIR, NEW JERSEY

## COVER FOR BOTTLE STOPPERS

Application filed May 9, 1925. Serial No. 29,258.

This invention relates to lids or protecting covers for bottle stoppers and for the exposed part of the pouring rim, flange or bead of the bottle and relates especially to paper covers of the cup type, protecting the stopper (e. g. the paper disc stopper employed as a closure for milk bottles) against dust and serving as a detector or indicator of any tampering with the contents of the bottle.

10 The cover may be made up of several sheets or plies of paper cemented together with a binder, or preferably as is set forth in the preferred embodiment hereunder single-ply paper is employed in making the cover. The 15 shape of the latter preferably is that of a cup or ramekin, with fluted or crimped sides forming the "skirt".

The usual method of fastening covers on milk bottles is by means of a wire ring which 20 clamps the crimped portion or skirt of the cover to the sides of the bottle below the mouth flange.

Covers which have a sufficient length of skirt to extend well below the mouth flange 25 may be used in accordance with the present invention but preferably I employ covers the crimped portion of which is somewhat shorter and when on the bottle extend barely below the mouth flange. A cover of this character presents a neat appearance and the amount of paper stock employed in making such covers is reduced.

In the present invention wire rings or metallic clamps are not used. The cover is impregnated or coated, or both impregnated and coated, either throughout or over a portion of the crimped area, with a sealing agent having a mild adhesion to glass. Preferably I employ a wax which is substantially non-adhesive to glass in conjunction with a saponifiable adhesive agent.

Thus I may employ hard waxes such as carnauba, candelilla, montan and shellac wax and the like having relatively high melting points, for example above 70° C. and preferably above 75° or 80° C.

When these hard waxes are melted and poured on glass in a thin layer it will be found on cooling that the wax peels or separates readily from the glass as for example

by gentle abrasion with the finger nail. This is a desirable quality to a certain degree in that it prevents fouling of the milk bottles through adhesion of the wax. The effect is quite different with softer and unsaponifiable waxes such as paraffin which when melted and poured on glass adheres rather tenaciously. Waxes of this character tend to foul the bottles.

On the other hand a cover carrying a binder of the aforesaid high melting point waxes not infrequently has too little adhesion and on slight swelling of the cover which may come from absorption of moisture from water or ice said cover may loosen sufficiently to be easily rotated around the mouth of the bottle. This would not be a particular objection if the rotation which may occur in handling did not have a tendency to cause the cover to spread by sliding upward slightly along the mouth flange. Covers which spread in this manner give the appearance that the contents of the bottle have been tampered with.

In the present invention I may incorporate with the high melting point wax having peeling properties, an adhesive substance such as dammar resin, copal or common rosin; the latter being very cheap and satisfactory. Cumaron resin might be used but would have the disadvantage of being unsaponifiable and therefore should particles of the binder adhere to the glass the hot soda ash solution used in washing the bottles in the dairy might not remove all the binding composition from the surface of the glass. Resin of this character is not recommended for the purpose but its use in some mixtures may be possible and is not precluded. The adhesive agent may be incorporated with the wax to the extent of 10 or 20 per cent or even in larger proportions depending on the degree of adhesion desired. A resinous body such as rosin or shellac both of which are very readily soluble in hot soda ash solutions has the advantage that if present in binder compositions they afford an emulsifying or disintegrating action when subjected to the hot alkaline solution and particles of the binder

55

60

65

70

75

80

85

90

95

100

sticking to the bottle therefore are removed in a relatively easy manner.

The resin and wax may be melted together to form the requisite mixture. In some cases 5 for example when using shellac which is not readily miscible with some waxes, blending agents may be required.

Metallo organic compounds of the waxes and resins likewise may be used or the mixture of wax and resin may be treated with a 10 small amount of base such as calcium or magnesium oxide or hydroxide to raise the melting point. Usually 2 or 3 per cent of the basic material suffices.

15 Such metallo organic compounds preferably and desirably are made by fusion rather than by precipitation, in order to save expense and avoid impurities which may be present when made by a wet method or precipitation procedures.

The cover is usually made of stiff strong paper but other grades of paper or special fibrous material may be employed. The paper should be treated with a lubricating 25 substance in order that it may be drawn, that is forced through dies to obtain the desired cup or ramekin shape. One or both sides of the paper therefore may have a coating of paraffin wax or other lubricating agent applied thereto prior to drawing. A desirable treatment proposed especially to be carried out in connection with the present invention is that of incorporating with the paper stock while in the beater engine a quantity of a 30 paraffin wax emulsion and adding a setting agent which causes the paraffin to precipitate throughout the particles of the pulp mass. Thus 2 or 3 per cent by weight of the paper stock may be introduced in this manner for 35 waterproofing purposes and larger proportions may be added to secure a lubricating effect to accomplish drawing to advantage. Such emulsions of wax may be made by agitating or grinding paraffin wax with water, 40 bentonite and a small amount of soap or alkali, or starch and caustic soda may be employed with the paraffin wax, or 5 or 10 per cent of stearic or oleic acid may be melted with the paraffin and this composition emulsified with a hot dilute aqueous solution of 45 caustic soda or ammonia. Preferably the paraffin emulsion is added to the beater engine at the time the paper stock is charged thereinto and after thorough admixing in the 50 usual manner, with or without the addition of rosin size or any other desired sizing agent, alum or other setting agent is added just before the charge is withdrawn.

The paper which is waterproofed in this 60 way also may be cut into discs of a size appropriate to fit into the mouths of milk bottles so as to form a closure for the bottles. Ordinarily discs of this character are water-proofed by applying to both surfaces a thin 65 coating of paraffin wax. In the present case

the wax is distributed through the mass of paper instead of being at the surface and a less greasy effect may be obtained with economy of wax.

The present invention in one form contemplates a bottle which is stoppered or closed by means of a paper disc containing paraffin emulsion as aforesaid and carrying a protecting cover preferably likewise water-proofed. 70

75 By applying paraffin wax in the paper in this manner the drawing operation may be carried out without having the surface of the paper saturated with wax, so that the binding wax described above when applied to the skirt of the cover does not become contaminated or diluted with objectionable amounts of paraffin.

80 The binding wax and resin composition may be applied to the cover by dipping the lower part of said cover in the molten mixture, or the covers may be nested and a column of such nested covers arranged with the skirts pointing downward. The molten composition is poured over the covers and a portion 85 of the wax collects on the exposed lower part of the skirt of each cover. Or the molten composition may be applied by spraying or in other ways. 90

95 In applying the covers to stoppered bottles the column of nested covers carrying the binding agent may be placed in a vertical container open at the bottom and provided with suitable means for removing one cover at a time and placing it on a bottle set just beneath the device. This vertical container is 100 preferably jacketed and is heated by steam or by steam blown into water contained in the bath. In some cases when special temperatures are desired the baths may contain 105 solvents such as alcohol or toluol with reflux condenser equipment so that on applying heat which ordinarily will be from the steam plant of dairy, the covers will not be heated above a certain desired temperature. 110

115 A quick-setting composition as the binding agent is important in most cases because the covering or capping of the bottles is carried out by machinery which is more or less automatic and the time allotted for the binding agent to set therefore may be only a few seconds. Ordinarily 6 to 10 seconds may not be exceeded. Preferably therefore the binding agent is maintained at a temperature only slightly above the softening or congealing 120 point. Some mixtures have so pronounced a lack in setting or hardening by cooling, especially when heated considerably above the melting point that much trouble arises in securing sufficient rapidity of set to allow their 125 use in dairy practice. By arranging to have the temperature of the heating bath at a definite relatively low point close to the softening or congealing point as aforesaid the rate of setting usually is substantially increased. 130

With larger proportions of resins which have less definite softening points this condition may be aggravated and preferably I employ a proportion of resin or resinate less in amount than the wax, that is the composition 5 contains a major proportion of wax. Paraffin wax alone is not satisfactory.

Various other substances may be employed in carrying out the present invention in replacement of the waxes in whole or in part or 10 in substitution for the resins or resinates, and when the color is not objectionable asphaltic substances such as gilsonite or other dark materials or coloring agents may be introduced. Metallo organic compounds such as 15 magnesium or calcium stearate, palmitate and the like also may be incorporated.

In the case of the latter addition mentioned I prefer to use products made by fusion rather 20 than by precipitation as in this manner magnesium or calcium stearate or palmitate may be very cheaply obtained in a state of purity or at least free from saline compounds or other substances which might accidentally 25 contaminate the contents of the bottle.

While paraffin wax by itself has the disadvantages set forth above, a considerable improvement results on mixing it with rosin. For example a mixture of equal parts of 30 rosin and paraffin melted together and applied to the skirt of the cover was found to be very waterproof and although there was some fouling of the glass the attached particles could be removed by washing; due no 35 doubt to the emulsifying character of the rosin intimately mixed with the wax. A mixture of 1 part of rosin to 3 parts of paraffin was removed from glass with greater difficulty.

40 A mixture of equal parts of cumaron resin, rosin and paraffin likewise did not offer difficulty of removal by washing with alkaline solutions. Congo resin 1 part, rosin 3 parts and paraffin wax 1 part was yellow in color 45 and did not foul glass.

A mixture of 5 parts rosin, 5 parts paraffin wax and 1 part of carnauba wax was found, like the foregoing to have a desirable cling or mild adhesion to glass but did not foul it. 50 The composition flaked off from glass on moderate pressure. Such a composition I consider superior to one composed largely or entirely of carnauba wax because of the slight cling without fouling and because the cost of 55 materials is so much less.

The foregoing examples have the desired cling or "grip" preventing rotation of the cover on the flange of the bottle on mild pressure, especially when a sufficient amount of 60 the binder is present. With respect to this proportion it may be noted that the paper may be simply impregnated with the composition or a larger amount may be employed so as to have a coating on the surface. The 65 latter is desirable especially since the single-

ply paper preferably employed in forming the cover when light in weight does not absorb enough of the binder on impregnation alone to make a firm seal in all cases. With heavier and more expensive paper this criticism 70 may not apply. However if the composition is not fouling it does not matter if an excess of the composition above that absorbed by the paper is present. Such additional amount of binder increases the strength 75 and firmness with which the cover is attached to the bottle.

The present invention therefore contemplates the employment of binders comprising rosin or other resin of an appropriate character incorporated with a soft wax such as 80 paraffin and preferably with a modifying wax such as carnauba. The proportions given above are useful ones since the mixture is low in cost and has the desired properties. 85

The carnauba wax may however be increased to secure a greater peeling effect. The rosin and paraffin may be varied for example twice as much rosin as paraffin may be employed. It is a matter of surprise that 90 paraffin wax which normally adheres to bottles in the manner indicated above, causing various difficulties, loses this property to a very considerable extent when incorporated with the rosin, particularly on the addition 95 of a small amount of a high melting point wax such as carnauba. The color of the mixture is satisfactory and the paper when thoroughly impregnated and slightly coated acquires a glossy finish. While the rosin and 100 paraffin by themselves do not give satisfactory results, when admixed as above and used as a binder for a single-ply cover excellent waterproofing results are obtained.

Covers impregnated with carnauba wax 105 alone as the binding agent or various other high melting point waxes are not particularly waterproof. Milk bottles are frequently packed in ice or handled under conditions of moisture which are severe, the bottles 110 oftentimes being actually submerged. When so submerged covers having carnauba wax as the binding agent will swell and loosen in the course of an hour or two. Sometimes the covers will loosen to such an extent that they 115 will separate from the bottle and float on the surface. With a rosin-paraffin-carnauba mixture in the proportion stated above a cover the skirt of which has been impregnated and coated therewith may be submerged 120 under water for a period of 12 hours or more without any material loosening of the skirt. This too despite the fact that the upper part of the cover over the top of the bottle which has had merely the usual glaze 125 of paraffin wax will be in a soft and swollen condition.

By impregnating the entire cover with the rosin-paraffin-carnauba mixture a remarkably complete waterproofing effect results 130

and the covers are especially permanent. In this case however it is better to use a larger proportion of carnauba wax than 5 or 10 per cent, preferably increasing to 20 or 30 per cent.

Other compositions are equal parts of dammar and paraffin wax; congo resin 1 part, rosin 3 parts, paraffin wax 3 parts; Congo resin 1 part, rosin 2 parts, paraffin wax 5 parts. A mixture of equal parts cumaron resin and paraffin wax was weaker.

The proportions given above are by weight. The covers in question it should be understood are made from a single sheet of paper, that is they are not composed of two or more sheets of paper cemented together. Such a single-ply cover is cheaper to make and the manufacturing difficulties connected with producing it are considerably less than with covers made with a plurality of layers of paper. A good strong type of paper heavy enough to stand handling incident to transporting milk bottles should be used. It may be glazed with paraffin, as heretofore employed in making the paper discs for closing milk bottles, or it may be waterproofed with emulsified wax as described above. A cover made with paper containing such emulsified wax may be referred to as waterproofed with or containing emulsified wax or wax which has been deposited from an emulsion by the employment of a suitable coagulating agent; such coagulation or setting preferably being carried out in the beater engine. A large part of the paper stock of the cover preferably is ground wood which may be admixed with wood pulp obtained by the sulphite or other processes. By employing a cover, the paper stock of which contains a considerable proportion of ground wood and impregnating a portion of the skirt or crimped part of the cover with the rosin-paraffin-carnauba wax mixtures aforesaid, it is possible to employ a comparatively short skirt which reaches only round the flange of the bottle and yet which when crimped into place has a strength and adhesion which could be secured with for example carnauba wax alone only by employing a much longer skirted portion.

Thus the invention in its preferred form relates to a cover for disc-closed bottles carrying a skirt-binder comprising a resin and waxy material, the latter preferably being a mixture of a cheap soft wax such as paraffin and a high melting point or hard wax such as carnauba; the latter being present in a proportion sufficient to substantially reduce adhesion to glass; there being however preferably sufficient adhesion to obtain a strong sealing effect when the cover with its binder softened by heat is crimped around the mouth of the bottle. There is thus involved the process which comprises melting together a resin which has the property of clinging to

glass and a high melting point wax which has the property of readily peeling from glass, the ratio of the resin and wax being in predetermined proportions to adjust the degree of cling and applying such composition to covers as a binding agent. Furthermore the invention comprises a milk bottle covered as aforesaid especially with a cover having a relatively short skirt reaching only to or just below the flange of the milk bottle; the length being preferably only sufficient to engage the jaws of the clamp when the cover is applied.

When water insoluble soaps or resinate are employed it should be noted that I prefer to employ products which have been made by fusion rather than precipitation in the wet way. By the latter procedure, which by the way is a relatively costly one, the coagulum is likely to occlude impurities such as the salts formed during the reaction. Preferably I employ stearates, palmitates, oleates, resinate and the like which have been made simply by fusion rather than by precipitation and thus avoid the presence in the covers of "chemicals" liable to cause suspicions on the part of laymen or of allegations by hostile interests.

Finally it may be noted that paraffin wax is extremely slow setting when employed alone, that it is rather greasy and exhibits a considerable degree of adhesion to glass. Rosin on the other hand sets fairly rapidly and is notably adhesive and sticky. Carnauba wax sets quickly and is substantially non-adhesive. It is surprising to find that the sticky qualities of rosin and the slow setting properties of paraffin wax are so considerably modified by their action one on the other and that carnauba or other high melting point waxes even in the small proportion of 10 per cent or thereabouts introduced into the mixture of rosin and paraffin exhibits such an unexpected behavior so that when used as a skirt-binder mild adhesion, substantial absence of greasiness, quick setting, strong binding effects and excellent water resistance result.

In using the term paper seal or binding agent it should be understood that it is not my purpose necessarily to hermetically seal the milk bottle. I desire to secure on the mouth of the bottle a cover which will prevent for all practical purposes, during the period that the bottle is exposed, the ingress of dust or impurities, also to make it difficult to tamper with the bottle without detection. Preferably therefore I do not use so abundant a coating of binder, nor paper of such a soft, yielding character that a hermetic seal results. The fluted or crimped portion of the cover or skirted part being made preferably of rather stiff strong paper ordinarily will permit the passage of air through various small openings along the sides of the skirt between it and

the bottle. The employment of a coating adequate to give sufficient strength as a binder for the skirt but not sufficient to cement the entire skirt in an air-tight manner to the glass renders the bottle more readily cleaned.

5 In any event it is preferable to impregnate solely the skirt of the cover or merely a part of said skirt when economy of material is desired. In such a case the upper part of 10 the cover as it rests on the upright bottle will be more or less easily permeable by air and a hermetic seal does not therefore result.

15 In the drawings which are of a conventional diagrammatic character, Figure 1 shows a bottle of the milk bottle type, the illustration being partly in elevation and partly in vertical cross section. Figure 2 shows a perspective view of a crimped or fluted paper cover or cup of the ramekin type and 20 Figure 3 shows such cup crimped about the mouth and rim of the bottle illustrated in Figure 1.

25 In the drawings A is a milk bottle having a paper disc closure or stopper B. C is a paper cap or cup having the smooth top across the mouth and upper surface of the bottle rim as shown and being bent or crimped around the bottle rim by the pressure of a crimping tool, the groove formed by which being shown 30 just below the bottle rim at D. E is the binding material composed of a mixture of resin and wax or other material within the range of equivalency of the present invention, such material being applied as an impregnum with 35 a certain amount preferably on the surface. The shaded portion of Figures 2 and 3 representing this binding material indicates either an impregnum or impregnated and coated areas. As shown the binder extends only part 40 way up the sides of the cup, but this depends on the length of the skirt and also on the manner of application of the binder. For example the caps may be nested so that only a portion of the skirt projects and the binder material may be poured over a column or stack 45 of these cups, the top portion C of the caps being uppermost. As the molten binder runs down over the sides of the stack of nested cups the exposed portion of the skirt will become 50 coated and perhaps impregnated. Afterwards the stacks may be kept warm for a time in a draining oven whereby excess of the binder drips off and more or less impregnation occurs. At the same time some of the 55 binder will creep upward along the skirt and the distance of travel by capillarity will depend upon the amount of binder present and the time and temperature of heating. With a sufficient application of binder and consider- 60 able heating the binder may run upward to the top of the skirt or even extend outward on to the horizontal portion of Figure 2.

65 In Figures 2 and 3 the fluted or crimped parts of the skirt are brought against and around the mouth of the bottle by the pres-

sure of a crimping or clamping device. The cover is warmed to soften the binder, then placed on the mouth of the stoppered bottle and the clamping pressure applied. Preferably this clamping effect is carried out by 70 means of a tool having a narrow edge in order that the clamping effect may be applied evenly despite the fact that the bottles may vary somewhat in size of mouth rim, etc. A clamping tool with narrow edge enables inequalities due to lack of uniformity in manufacture 75 of bottles to be taken up adequately.

The paper employed in making the cup C preferably is ordinary fibre paper of strength sufficient to resist the conditions of handling 80 and transportation. Hence paper which is fairly stiff and tough is desirable. Paper of this character tends to resist crimping about the bottle rim and after the clamp is released tends to spring away from the bottle. With 85 paraffin wax due to its slow set and lack of strength I have not been able to employ strong paper effectively. Even after the clamp has been applied for 5 or 10 minutes paper of this desirable character refuses to retain its shape 90 firmly on the bottle rim and especially when in contact with moisture I observed the crimped portion expand and the cap becomes loose and may fall off.

95 Hence in accordance with the present invention I propose, as I have heretofore stated, to utilize a binding composition which permits of the crimping operation to be accomplished in from say 6 to 10 seconds or in any event during a very short interval of time 100 so that bottles may be handled in large numbers in the dairy with the least possible expenditure of time. By employing a resinous substance, adhesive to glass, in conjunction with waxy material a good grip is produced 105 along the line D where the crimping tool is applied. Fillers in the binding composition are preferably avoided as they simply act as loading agents which detract from the strength and the problem of finding a substance which is cheap and yet has strength and waterproof qualities is difficult at best without the addition of adulterating substances such as fillers. However in some cases 110 when special colors are desired pigment-fillers 115 may be used.

When crimped into place the cup C preferably does not form projecting fins but simply the ordinary creases and tucking crimps under the shoulder of the bottle neck or rim or flange that will naturally result from such contraction and compression due to the crimping tool. Furthermore the amount of binder which I preferably employ is not sufficient to fill all the little creases around the neck of the bottle due to such crimping. Where the fluting is folded over and flattened out against the bottle due to the stiffness of the paper and desirability of using only a sufficient 120 amount of binder to give the requisite 125

strength, there will be occasional little channels through which air may pass and possibly at times a slight amount of moisture. Such fine channels do not offer any difficulty due to ingress of water when the bottle is submerged and even if water should penetrate in this manner it cannot pass the true closure or stopper B. On the other hand such minute channels act as equalizers of pressure on the 5 two surfaces of the closure B which is sometimes desirable. By having the binder applied only along the skirt of the cap C the upper part remains more or less permeable to air. Even when given the thin paraffin wax 10 finish on both sides following the treatment ordinarily employed in the case of the paper disc closure B it will be found that moisture will be absorbed in the interior of the paper sheet when the cup is submerged. There is 15 thus a change in volume and certain stresses are set up which tend to increase the spring or tendency of the skirt of the cup to open, leaving the rim of the bottle. This loosening may be slight, just sufficient to cause the cup 20 to be easily rotated around the rim of the bottle or it may be sufficient so that the cap when submerged in water will come off entirely and float to the surface. Rosin and various resins appear to be far more effective 25 as waterproofing agents than waxes. The resins however by themselves are sticky and oftentimes not workable for various other reasons but when incorporated with wax qualities are obtained from the composition 30 which do not appear in either taken separately. Thus for example both paraffin wax and carnauba wax used by themselves as binders are quickly loosened when wet, in the case of cap covers the upper part of which is not 35 impregnated but simply glazed with a wax coating. Under these conditions the moisture which penetrates into the fibre of the paper forces the crimped portion away from the rim of the bottle with undesirable loosening. 40 This may occur in fifteen minutes to an hour. Bottles frequently while in transit are under packed ice or in moist conditions for a period of ten or twelve hours and I have found the resin-wax mixture previously described offers 45 the necessary waterproof qualities in a binder 50 for the skirt to meet such requirements.

While I have stated the resin-wax mixture is preferably applied in the molten condition as an impregnating and coating composition 55 I do not limit myself thereto but may resort to the employment of resin and wax emulsions which may be incorporated in the ground wood and wood pulp mixture preferably employed in making the paper stock. 60 Such deposited resin and wax obtained from appropriate emulsions thereof, as for example an emulsion of paraffin wax and carnauba wax in rosin soap solution does not form a part of the preferred embodiment of the present 65 invention. By the impregnating method

described the binder can be applied locally to the skirt of the cap where it is most needed whereas by the emulsion method the binder is distributed throughout the paper material uniformly and is less effective.

It will be noted therefore by such partial or localized impregnation no attempt is made to produce a cover which is airproof and waterproof although by complete impregnation with the rosin-wax mixture extremely effective resistance to water is obtainable. Such treatment is not necessary however as the cup does not function as a stopper but merely as a stopper cover. Complete impregnation of the cup adds to the cost of material and furthermore covers impregnated throughout with rosin-wax mixtures tend somewhat more to stick together in the 70 cupping machine cup magazine and also to the plunger used to push the cover onto the bottle. By impregnating simply the skirt and not the top of the cover this difficulty is 75 avoided.

What I claim is:—

1. A single-ply, skirted paper cap made from paper stock, containing a considerable proportion of ground wood, said cap carrying a binder of a quick-setting wax.
2. A single-ply, skirted paper cover made from paper stock, containing a considerable proportion of ground wood, said cover carrying a binder of a quick-setting wax.
3. A single-ply, skirted paper cover made from paper stock, containing a considerable proportion of ground wood, said cover carrying a binder containing a quick-setting wax and resin mixture.

CARLETON ELLIS.

105

110

115

120

125

130